

## UNITED STATES PATENT OFFICE

1,970,467

## PROCESS FOR WORKING UP FERRO-VANADIUM CONTAINING PRODUCTS

Eugen Mayr, Lautawerk/Lausitz, Germany, assignor to Otavi Minen- und Eisenbahngesellschaft, Berlin, Germany, a company of Germany

No Drawing. Application October 25, 1933, Serial No. 695,215. In Germany October 28, 1932

2 Claims. (Cl. 75—17)

This invention refers to the treatment of vanadium containing products, especially vanadium containing slags.

As is well-known the production of ferrovanadium is preferably effected by aluminothermic reduction of vanadic acid. In this way products are obtained which in addition to alumina, magnesia, a little iron, silicic acid and other impurities have a not inconsiderable vanadium content, 10 and inasmuch represent a valuable material.

The working up of these products containing vanadium on the one hand to a useful ferrovanadium, and on the other hand to a marketable corundum however entails great difficulties.

15 Attempts have been made in this respect to fuse the slag from the aluminothermic reduction of vanadic acid in the electric furnace with addition of various substances such as for example bauxite, lime, hammer scale, or cast iron shavings or filings and carbon or coal. Operations carried out thus have not led to any useful result. The vanadium content of the fused metal alloy was too small for a marketable ferrovanadium and was uncertain; the silicon amounted 20 up to 6%, and the carbon content up to 10%. Also the corundum produced in this way contained more or less much carbide. The furnace operation was irregular and therefore difficult to control.

30 It was not possible either however to work up the metal alloy obtained by acid treatment, since this alloy is practically and economically insoluble in acid. For the most part, therefore, the expensive disintegration by means of soda was used.

The purpose of the present invention is to remove these disadvantages.

According to the invention the products containing vanadium are, without any other addition, than reducing materials, fused in an electric furnace, having for example a magnesite lining and a magnesite bottom. In this way an alloy having a high content of ferrovanadium is obtained and a corundum which is practically free 40 from vanadium and carbon and therefore marketable. The corundum and the metal alloy can be separated very simply and the corundum conveniently drawn off. The furnace operation is perfectly normal and therefore can be easily 45 controlled.

As already stated the metal alloy obtained is rich in vanadium and indeed contains about 70% and more of this metal, together with a little silicon and about 8% of carbon.

50 This metal is comminuted or ground and heat-

ed to incandescence in order to oxidize the metal, during which operation the vanadium is converted into  $\text{VaO}_2$  and the carbide is burnt off as well. A practically pure mixture of oxides of vanadium and iron results. This is fused, for example 60 aluminothermically, to a practically pure ferrovanadium.

A further advantage of the process is also to be seen in the fact that the vanadium is not converted into its highest oxidation stage during the 65 oxidizing heating of the ferrovanadium. This is very favourable since this lower oxide requires less aluminium during the aluminothermic process.

The conversion of the metals into their oxides 70 can be dispensed with if the comminuted alloy can be added to a process in which the oxidation is effected.

What I claim is:—

1. A process for working up vanadium containing slags consisting in fusing the said slags with the only addition of reducing agents in an electric furnace, oxidizing the resulting impure ferrovanadium by heating the same to about incandescence in an oxidizing atmosphere and recovering a pure ferrovanadium in a suitable manner. 75

2. A process for working up vanadium containing slags consisting in fusing the slags with the only addition of reducing materials in an 85 electric furnace, comminuting the resulting impure ferrovanadium, oxidizing the same by heating it to about incandescence in an oxidizing atmosphere and recovering a pure ferrovanadium by aluminothermic reduction. 90

EUGEN MAYR.

95

100

105

110